

Jan. 8, 1935.

R. L. PEEK, JR

1,987,416

SUBMARINE TELEGRAPH CABLE

Filed Feb. 20, 1929



INVENTOR  
R. L. PEEK JR.  
BY  
*J. W. Schmied*  
ATTORNEY

## UNITED STATES PATENT OFFICE

1,987,416

## SUBMARINE TELEGRAPH CABLE

Robert L. Peek, Jr., Union, N. J., assignor to Bell Telephone Laboratories, Incorporated, New York, N. Y., a corporation of New York

Application February 20, 1929, Serial No. 341,368

10 Claims. (Cl. 173—264)

This invention relates to submarine telegraph cables and more particularly to deep sea submarine cables of light and simplified construction for use under conditions where a light service demand necessitates low cost of construction and laying.

It has been found that there is a demand for telegraph service between points, separated by deep oceanic waters, where the traffic would be too low to justify the expense of laying a submarine cable of the type in which an outer armoring is placed about the insulation to provide the necessary tensile strength of the cable during laying operations or during lifting operations for repairs.

It has before been proposed to eliminate the outer armoring from deep sea cables and to place light, steel armor wires directly about the conductors, thereby providing a metallic core of sufficient tensile strength to sustain the weight of the cable while it is not resting on the sea bottom. It has also been proposed to substitute for the usual outer steel armoring a wrapping of hemp or like material which would provide the necessary tensile strength during the laying operations. It has furthermore been proposed to substitute for some or all of the outer steel armor wires strands of light metal, such as aluminum, or of more highly conducting metal, such as copper.

In accordance with the present invention a deep sea cable is constructed with a central conductor of one or more non-magnetic metals or alloys of sufficient conductivity to provide for a limited traffic and having such light weight and high tensile strength that the conductor is capable of sustaining the total weight of the cable during the process of laying in the sea so that an outer armoring around the insulation will not be required for this purpose, even at depths as great as 2 to 2½ nautical miles.

The central conductor in accordance with this invention may be composed entirely of hard drawn aluminum or of an aluminum alloy of high tensile strength, which will have sufficient conductivity to serve in a low speed telegraph system. The conductor may furthermore comprise a combination of strands, some of which are made of aluminum or of the alloys thereof, referred to, and others of which may be either of hard drawn copper or a copper alloy of high tensile strength. By such a combination of metals the average conductivity of the stranded conductor may be high enough to meet the particular service requirements and its strength at the same time may be

maintained at a value which will permit of laying in comparatively deep water without danger of breakage.

In the following description reference will be made to the accompanying drawing which shows a portion of a submarine cable to which the present invention may be applied.

In the design of submarine cables the question of cost is extremely important. Since the cost is directly related to the dimensions of the several elements within the cross section of the cable, it is imperative to consider with the utmost care even the slightest dimensional changes in the cross section as well as the choice of materials. This is especially true in the case of telegraph cables where the service is not exacting and the revenue low, that is, where the traffic amounts to say only 200 words a minute at simplex operation over distances of 1000 miles or more. This class of service may of course include cables of somewhat shorter length with a corresponding increase in traffic capacity.

Cables of this type must therefore be reduced to minimum dimensions and must be of the simplest possible construction. Due to the low signaling frequency, loading of the conductor with magnetic material is not necessary and the skin effect is negligible. For the deep sea portions of such cables the outer armoring should also be dispensed with and a braiding may take its place for the protection of the insulation. It is consequently necessary to construct the cable with a metallic conductor, which not only meets the traffic requirements, but which also is capable of sustaining the weight of the cable in water during laying operations over depths which frequently may be as great as 2½ miles or even more, which means that when the usual safety factor of 2 to 3 is applied, the cable must be able to carry its own weight in water at a hypothetical depth as great as 5 to 7 miles. This hypothetical depth will be referred to hereinafter as the "breaking length" of the cable, or of any particular strand thereof, and is the length which the cable or strand is just able to sustain at the verge of breaking when it is suspended vertically in water.

To provide a given resistance of the conductor per unit length of cable, as required by the estimated traffic, the designer may choose from a limited number of metals for the conductor. The cost of the metal proper is of course important and the overall diameter of the conductor, which for a given resistance depends upon the specific conductivity of the metal, greatly influences the

amount of insulation which must be placed around the conductor and thus the cost of the insulation as well as that of the outer braiding. The traffic capacity of a cable of the type 5 under consideration is roughly inversely proportional to the product of the electrical resistance and the electrical capacitance of the cable. For a given insulating material the capacitance is proportional to the ratio of outer to inner diameter of the insulation. Hence for a given capacitance the outer diameter of the insulation must be proportional to the diameter of the central conductor, which determines the inner diameter of the insulation. The electrical resistance of the cable is inversely proportional to the cross sectional area of the conductor and directly to the resistivity of the metal or metals composing the conductor. From these considerations it is apparent that the substitution of a metal of 15 higher resistivity for one of lower resistivity in the central conductor will necessitate an increase in the diameter of the conductor and a proportional increase in the outer diameter of the insulation, and hence results in a considerable increase in the total amount of insulation and in the cost of the cable, when a given traffic capacity is to be maintained.

Therefore, when it is desired that the central conductor of a cable should have sufficient strength to itself support the cable in water, thus eliminating the necessity of an outer metallic armoring, it is of the greatest importance that such a conductor should have the lowest possible average electrical resistivity consistent 30 with such strength.

The choice of metals thus involves the consideration of their tensile strength in relation to their weight per unit volume in water, which relation is expressed by the breaking length of 40 the metals. The weight of the insulating materials and of the braiding materials may be disregarded in these considerations since their specific gravity usually is close to 1 and they therefore do not add to the weight of the conductor in water.

The following table contains, beside other data, the conductivity in per cent of that of pure annealed copper and the breaking length of a 50 number of metals and alloys which are suitable for submarine conductors.

Table I

| Material                | Conductivity (%) | Specific gravity in water | Tensile strength (lbs./sq. in.) | Breaking length (nauts.) |
|-------------------------|------------------|---------------------------|---------------------------------|--------------------------|
| Annealed copper         | 100              | 7.9                       | 15,000                          | .72                      |
| Hard drawn copper       | 97               | 7.9                       | 60,000                          | 2.89                     |
| Cadmium bronze          | 85               | 7.9                       | 78,000                          | 3.76                     |
| Hard drawn aluminum     | 60               | 1.7                       | 28,000                          | 6.82                     |
| Aluminum alloy No. 2    | 55               | 1.7                       | 48,000                          | 10.89                    |
| Aluminum alloy No. 1    | 35               | 1.8                       | 70,000                          | 14.9                     |
| Elektron                | 35               | .8                        | 32,000                          | 15.8                     |
| High carbon steel No. 1 |                  | 6.9                       | 120,000                         | 6.62                     |
| High carbon steel No. 2 |                  | 6.9                       | 180,000                         | 9.9                      |

Aluminum alloy No. 2 contains aluminum and 65 less than 2% of magnesium and silicon. Aluminum alloy No. 1 consists of approximately 94.3% aluminum, 4% copper, 0.8% manganese, 0.6% magnesium and 0.3% silicon. These compositions are representative of two distinct types 70 of well known aluminum alloys.

Hard drawn aluminum and alloy No. 2 combine a fairly high conductivity with high breaking length and may therefore, in accordance with the invention, be used exclusively for the conductor at a depth of more than 2 miles and where

the traffic is low enough to not require an excessively large diameter of the conductor with a consequent unreasonable cost of insulating material. In order to reduce the size of the conducting strand, when desired, high conductivity metals such as hard drawn copper or cadmium bronze may be used, in accordance with this invention, with either hard drawn aluminum or alloy No. 2 to provide conductors of sufficient breaking length for different laying depths.

As an example, a cable may be assumed, such as shown in the drawing, where the conductor 10 is surrounded by a heavy layer of insulation 11 of any suitable material which in turn is protected by any suitable braiding 12 of light and tough, water resistant material such as hemp. The conductor may consist of 7 strands of equal size and of hard drawn copper and aluminum alloy No. 2. The number of strands of each material may be determined from the left hand section of Table II below in accordance with the requirements for conductivity and breaking length.

Table II

| Conducting core of hard drawn copper and aluminum alloy No. 2 |                   |                                 |                                                | Conducting core of hard drawn copper and high carbon steel No. 2 |                                  |                                                |                            |
|---------------------------------------------------------------|-------------------|---------------------------------|------------------------------------------------|------------------------------------------------------------------|----------------------------------|------------------------------------------------|----------------------------|
| No. of strands                                                | Hard drawn copper | Alumi-<br>num<br>alloy<br>No. 2 | Break-<br>ing<br>length<br>of core<br>(nauts.) | No. of strands                                                   |                                  | Break-<br>ing<br>length<br>of core<br>(nauts.) | Con-<br>ductiv-<br>ity (%) |
|                                                               |                   |                                 |                                                | Hard<br>drawn<br>copper                                          | High<br>carbon<br>steel<br>No. 2 |                                                |                            |
| 7                                                             |                   | 0                               | 2.89                                           | 97                                                               | -----                            | -----                                          | -----                      |
| 6                                                             |                   | 1                               | 3.17                                           | 91                                                               | -----                            | -----                                          | -----                      |
| 5                                                             |                   | 2                               | 3.51                                           | 85                                                               | 9                                | 1                                              | 3.52                       |
| 4                                                             |                   | 3                               | 3.98                                           | 79                                                               | 8                                | 2                                              | 4.19                       |
| 3                                                             |                   | 4                               | 4.65                                           | 73                                                               | 7                                | 3                                              | 4.85                       |
| 2                                                             |                   | 5                               | 5.66                                           | 67                                                               | 6                                | 4                                              | 5.45                       |
| 1                                                             |                   | 6                               | 7.36                                           | 61                                                               | 3                                | 7                                              | 5.56                       |
| 0                                                             |                   | 7                               | 10.85                                          | 55                                                               | -----                            | 7.56                                           | 30-36                      |

For the sake of comparison, Table II also contains data for the conductivity and breaking length of conductors of 10 strands made of hard drawn copper and high carbon steel No. 2 of 45 high tensile strength, the entries being so arranged that the breaking lengths of the copper-steel conductors closely approximate those of corresponding copper-aluminum conductors in the left hand portion of Table II. The conductivity of steel is largely dependent upon the carbon content and may vary up to 10% of that of copper; this variation affects the total conductivity as indicated by the limiting figures in the table.

From a comparison of the conductivity of the two types of conductors at similar breaking lengths, it becomes apparent that the advantage of the copper-aluminum conductor over the copper-steel conductor increases as the breaking length increases. Thus at a laying depth of 2 miles, corresponding to a breaking length of about 5.5 miles which frequently is required in oceanic waters, the difference in conductivity is more than 5%, so that by the use of the aluminum alloy in place of steel the cross sectional area of the conductor may be reduced by 5% and a saving in insulating material of a much higher percentage is attained. Calculations furthermore show that the weight ratio in water of the copper-aluminum and copper steel conductors of 70 breaking length of 5.5 miles is as 3.47 to 7.5 or a reduction in weight of more than 50%. This of course means much easier handling during the laying operation, lighter machinery, and the need of only comparatively small boats. Such a reduc- 75

tion in weight of course is of extreme advantage at great laying depths where a very great length of cable must be held suspended during the laying operations.

- 5 Similar considerations show that cadmium bronze may be used instead of copper in a cable such as described above. For a given breaking length a smaller proportion of aluminum alloy No. 2 may then be used or this alloy may be re-  
10 placed by hard drawn aluminum. Various other combinations of copper, aluminum and their alloys are possible within the scope of this invention. The desired combination may be attained with the strands of equal size, or of different  
15 sizes, or in any other desirable manner, as for example by drawing the two desired metals in the proper proportions into a single strand. It is also contemplated that a given cable may have different sections with different combinations of  
20 metals making up the central conductor and may be of different constructions. Thus the proportion of high conductivity metal to high tensile strength metal may be made smaller in sections at smaller depths than in those at greater depths,  
25 and shore sections may furthermore be armored in the usual manner with an outside armoring.

In the case of cables to be placed in tropical waters and in which the insulation is protected from teredo attack by a sheathing of metal the weight of this sheathing must of course be taken into consideration in determining the load on the core, since this sheathing usually does not add to the tensile strength of the cable. The outer braiding, on the other hand may be of such design and materials that it would aid materially in supporting the cable during lifting or laying operations, so that the strength requirements of the conducting core may be reduced.

What is claimed is:

- 40 1. A signaling cable for laying in the sea to depths of about two miles or more, comprising a central nonmagnetic composite conductor and insulating material surrounding said conductor, characterized in this that the metallic composition of said conductor comprises separate aluminum and cupreous metals in such proportions that the average conductivity of the total conductor is more than 50% of that of annealed copper and that the breaking length of said conductor is  
45 about four miles or more so that the conductor is capable of safely sustaining its own weight during laying in the sea to said depth.

2. A signaling cable having sufficient tensile strength for safe laying in the sea to depths of about two miles or more, comprising a central non-magnetic composite conductor and an insulating sheathing surrounding said conductor, said conductor being composed of separate aluminum and cupreous metals in proportions such that it has an average conductivity of more than 50% of that of annealed copper and has a breaking length of about four miles or more so as to be capable of sustaining its own weight during laying in the sea to said depth without the support of an outer armoring.

3. A deep sea signaling cable, comprising a conducting center and a surrounding insulating sheath, said conducting center being composed

of separate elements of aluminum and copper in such proportions of volume that the average conductivity of said center is at least 50% of that of annealed copper and that the breaking length is about four miles or more.

4. In a submarine cable, a metallic core and an insulating sheathing surrounding said core, said core comprising a strand of aluminum alloy containing manganese and silicon in an amount not to exceed 2%.

5. A submarine signaling cable for laying at great ocean depth, comprising a metallic core and insulating sheathing thereabout, said core comprising at least one strand of a metal with copper as its main constituent and another metallic strand with aluminum as its main constituent and having a conductivity of more than 35% of that of annealed copper, and the proportion of one kind of strand to the other kind of strand being such that said core has a breaking 20 length of about four miles or more.

6. A deep sea cable for laying at a depth of about two miles or more, comprising a central conductor for telegraph signaling and a sheathing therearound having high insulation resistance 25 in sea water, said conductor including at least one strand of a metal with copper as its main constituent and another strand of an aluminum alloy having a conductivity of more than 35% of that of annealed copper, and the proportion by 30 volume of said metal to said alloy in said conductor being such that it has a breaking length in the sea of more than five miles.

7. In a submarine cable, a metallic core and an insulating sheathing thereabout, said core 35 comprising at least one strand of cupreous metal and another strand of aluminum alloy containing manganese and silicon in an amount not to exceed 2%.

8. A submarine cable core having a safe breaking length for laying in the sea to a depth of about two miles or more, comprising a conducting center having a conductivity of at least 50% of that of annealed copper and an insulating sheath enveloping said center, said conducting 45 center being non-magnetic and composed of at least 20% by volume of an aluminum metal and less than 80% by volume of a cuprous metal.

9. In a deep sea submarine signaling cable, a non-magnetic metal core and an insulating 50 sheath about said core, said core being composed of a continuous element of cupreous metal and another continuous element of aluminum metal and having sufficient breaking length to sustain the weight of the cable without the aid of armoring during laying in the sea to depths of about two miles or more with a safety factor of about 55 two or more.

10. An armorless deep sea signaling cable, comprising a conducting center and a surrounding 60 sheath having high insulating resistance under sea bottom conditions, said conducting center being composed of separate elements of aluminum and copper in such proportions of volume that the average conductivity of said center is at least 65 50% of that of annealed copper and that the breaking length is about four miles or more.

ROBERT L. PEEK, JR.